

1

3,672,878

ALUMINUM OFFSET PRINTING PLATE  
Adolf Teubler, Uedorf, near Bonn, and Paul Eversheim,  
Bonn, Germany, assignors to Vereinigte Leichtmetall-  
Werke G.m.b.H., Bonn, Germany  
No Drawing. Filed Sept. 24, 1969, Ser. No. 860,805  
Claims priority, application Germany, Sept. 27, 1968,  
P 17 83 066.9, June 9, 1969, P 19 29 146.4  
Int. Cl. C22c 21/04

U.S. Cl. 75—141

4 Claims

## ABSTRACT OF THE DISCLOSURE

An aluminum printing plate for use in offset roller plat-  
ing is made of an aluminum base alloy including the  
following alloying components:

|           | Percent  |
|-----------|----------|
| Magnesium | 0.8-2.5  |
| Silicon   | 0.2-0.4  |
| Manganese | 0.8-1.4  |
| Copper    | 0.05-0.3 |
| Iron      | 0.2-0.6  |
| Zinc      | 0.01-0.2 |
| Aluminum  | Balance  |

## BACKGROUND OF THE INVENTION

A material consisting of aluminum as the base ma-  
terial with a purity of 99% and more has already been  
used for printing plates in offset printing, particularly for  
single-color prints. However, these plates were not suitable  
for so-called roller offset printing. If the aluminum plate  
or sheet has a tensile strength of about 16 to 18 kp./mm.<sup>2</sup>,  
as required to obtain the necessary stability and rigidity,  
the danger of tearing of the sheet at the sharp-angled  
clamping edges is substantial. These edges, however, are  
necessary for the narrow, tight clamping of the offset plates  
on the rollers of the printing machine. A tearing of the  
sheet is particularly obnoxious if it occurs—not during the  
initial angling of the edges or during the clamping but—  
by virtue of the centrifugal force during actual operation  
such as results from the high rotation speed of the print-  
ing cylinder.

It is therefore an object of the present invention to pro-  
vide for printing plates for offset roller printing processes  
which (a) have a high rigidity to be stored in upstanding  
position and also to assure form stability during high  
rotation speeds; (b) are sufficiently flexible to permit that  
the plates, when clamped on the printing cylinder, con-  
form smoothly and exactly to the surface of the cylinder;  
and (c) have good angling properties so as to prevent  
tearing during the acute angle folding or subsequently  
when subjected to a high tensile stress.

## SUMMARY OF THE INVENTION

These objects are met by an offset printing plate which  
consists of an aluminum base alloy and includes the fol-  
lowing alloying components in the following percentages  
by reference to the weight of the total composition

|           | Percent  |
|-----------|----------|
| Magnesium | 0.8-2.5  |
| Silicon   | 0.2-0.4  |
| Manganese | 0.8-1.4  |
| Copper    | 0.05-0.3 |
| Iron      | 0.2-0.6  |
| Zinc      | 0.01-0.2 |
| Aluminum  | Balance  |

## DESCRIPTION OF THE PREFERRED EMBODIMENTS

In addition to the components listed above, the print-

2

ing plate of the invention may also include 0.01 to 0.05%  
titanium, and 0.001 to 0.005% boron.

The preferred composition for the printing plates  
would be as follows:

|           | Percent |
|-----------|---------|
| Magnesium | 1.5     |
| Silicon   | 0.3     |
| Manganese | 1.1     |
| Copper    | 0.15    |
| Iron      | 0.4     |
| Zinc      | 0.1     |
| Aluminum  | Balance |

Another preferred embodiment would be constituted as  
just described, but would additionally include 0.03% ti-  
tanium and 0.003% boron.

The general mechanical properties of the alloys used  
according to the invention for the printing plate appear  
from the following combination:

|                                                         | Soft condition |
|---------------------------------------------------------|----------------|
| Yield point: $\delta_{0.2}=16-24$ kp./mm. <sup>2</sup>  |                |
| Tensile strength: $\delta_B=17-22$ kp./mm. <sup>2</sup> |                |
| Elongation: $\delta_5=15-30\%$                          |                |

### Intermediate hard condition

|                                                         |
|---------------------------------------------------------|
| Yield point: $\delta_{0.2}=16-24$ kp./mm. <sup>2</sup>  |
| Tensile strength: $\delta_B=20-28$ kp./mm. <sup>2</sup> |
| Elongation: $\delta_5=8-15\%$                           |

These properties will afford a high rigidity, permitting  
to store the plates in upstanding position. It will also as-  
sure that the plates are not subject to deformation during  
the high rotation speeds.

The alloy furthermore has a sufficient flexibility. The  
plates therefore, when clamped onto the printing cylinder,  
can be made to conform completely to the cylinder.

These alloys also give the printing plates a good angling  
property. As a result, the plates will not be subject to  
tearing when they are clamped onto the cylinder and the  
acute angle edges are being formed. Also, during opera-  
tion, when the plates are subject to substantial tensile  
stress, they will not have a tendency to tear at the clamped  
edges.

Preferably, the aluminum base plates formed as de-  
scribed are provided on both major faces with plating  
layers. These layers may be applied by conventional  
roller plating processes. The plating may for instance con-  
sist of pure aluminum of a degree of purity between 99  
and 99.9%. Preferably, the plating layer has a thickness  
between 2 and 16% relative to the thickness of the entire  
plate. The thickness just stated for the layer applies to  
each separate plating layer. The offset plate may be  
anodized. Particularly preferred would be an aluminum  
plating of a purity of about 99.4%.

However, the plates most preferably are provided with  
plating layers on both major faces which layers are com-  
posed like the principal material, that is, the aluminum  
coating contains the same components as the core mate-  
rial but in different percentages. The total plating layers  
may for instance have a thickness of about 8% relative  
to the total thickness of the entire plate. The total plate  
may for instance after plating have a thickness of 0.50  
mm.

The following examples will further illustrate the  
invention.

### EXAMPLE 1

An aluminum offset printing plate was formed by plating  
in a roller plating process an aluminum core with  
layers having a combined thickness of about 8% of the  
total thickness of the plate. The total thickness was 0.50  
mm.

The composition of the aluminum alloy employed was as follows (all percentages relative to weight of the total composition):

| Core element:   | Percent |    |
|-----------------|---------|----|
| Copper          | 0.15    | 5  |
| Manganese       | 1.10    |    |
| Magnesium       | 1.12    |    |
| Silicon         | 0.30    |    |
| Iron            | 0.45    |    |
| Zinc            | 0.05    | 10 |
| Titanium        | 0.01    |    |
| Boron           | 0.003   |    |
| Aluminum        | Balance |    |
| Plating layers: | Percent | 15 |
| Copper          | 0.01    |    |
| Manganese       | 0.02    |    |
| Magnesium       | 0.01    |    |
| Silicon         | 0.18    |    |
| Iron            | 0.41    | 20 |
| Zinc            | 0.07    |    |

The properties obtained with this type of plate were as follows:

Yield point: 21.0 kp./mm.<sup>2</sup>

Tensile strength: 24 kp./mm.<sup>2</sup>

Elongation: 8%

#### EXAMPLE 2

The same type of printing plate was formed as described in Example 1. However, the composition of the core material and plating layers was as follows:

| Core material:  | Percent |    |
|-----------------|---------|----|
| Copper          | 0.10    |    |
| Manganese       | 0.85    | 35 |
| Magnesium       | 2.20    |    |
| Silicon         | 0.30    |    |
| Iron            | 0.45    |    |
| Zinc            | 0.07    |    |
| Titanium        | 0.012   | 40 |
| Boron           | 0.003   |    |
| Aluminum        | Balance |    |
| Plating layers: | Percent |    |
| Copper          | 0.01    | 45 |
| Manganese       | traces  |    |
| Magnesium       | 0.02    |    |
| Silicon         | 0.20    |    |
| Iron            | 0.41    |    |
| Zinc            | 0.08    | 50 |
| Aluminum        | Balance |    |

The printing plate of this example had the following properties

Yield point: 24 kp./mm.<sup>2</sup>

Tensile strength: 28 kp./mm.<sup>2</sup>

Elongation: 6%

#### EXAMPLE 3

An offset printing plate was again formed as described in Example 1 with the following difference in the composition of the alloys:

| Core material: | Percent |    |
|----------------|---------|----|
| Copper         | 0.14    |    |
| Manganese      | 1.12    | 65 |
| Magnesium      | 1.6     |    |
| Silicon        | 0.25    |    |
| Iron           | 0.35    |    |
| Zinc           | 0.06    |    |
| Titanium       | 0.011   | 70 |
| Boron          | 0.002   |    |
| Aluminum       | Balance |    |

| Plating layers: | Percent |
|-----------------|---------|
| Copper          | 0.002   |
| Manganese       | 0.005   |
| Magnesium       | 0.004   |
| Silicon         | 0.20    |
| Iron            | 0.40    |
| Zinc            | 0.03    |
| Aluminum        | Balance |

The printing plate of this example had the following properties:

Yield point: 13 kp./mm.<sup>2</sup>

Tensile strength: 23 kp./mm.<sup>2</sup>

Elongation: 18%

The printing plates of all three examples as above described had excellent properties for roller offset printing and were generally considered acceptable by the printers.

We claim:

1. An aluminum printing plate for use in offset roller printing, the plate consisting of an aluminum base alloy including the following alloying components:

|           | Percent  |
|-----------|----------|
| Magnesium | 0.8-2.5  |
| Silicon   | 0.2-0.4  |
| Manganese | 0.8-1.4  |
| Copper    | 0.05-0.3 |
| Iron      | 0.2-0.6  |
| Zinc      | 0.01-0.2 |
| Aluminum  | Balance  |

2. The printing plate of claim 1 which includes 0.01 to 0.05% titanium and 0.001 to 0.005% boron.

3. The printing plate of claim 1 wherein the aluminum base alloy includes the following alloying components in the following percentages:

|           | Percent |
|-----------|---------|
| Magnesium | 1.5     |
| Silicon   | 0.3     |
| Manganese | 1.1     |
| Copper    | 0.15    |
| Iron      | 0.4     |
| Zinc      | 0.1     |

4. The printing plate of claim 3, which includes 0.03% titanium and 0.003% boron.

#### References Cited

##### UNITED STATES PATENTS

|           |        |               |           |
|-----------|--------|---------------|-----------|
| 3,490,955 | 1/1970 | Winter et al. | 75-141 X  |
| 2,240,732 | 5/1941 | Wood          | 101-458 X |
| 2,290,016 | 7/1942 | Bonsack       | 75-141    |
| 2,290,025 | 7/1942 | Bonsack       | 75-141    |
| 2,922,731 | 1/1960 | Rutemiller    | 75-141 X  |

##### FOREIGN PATENTS

|           |        |          |
|-----------|--------|----------|
| 1,206,596 | 9/1965 | Germany. |
|-----------|--------|----------|

L. DEWAYNE RUTLEDGE, Primary Examiner

E. L. WEISE, Assistant Examiner

##### U.S. CL. X.R.

101-459